

# UNITED STATES PATENT OFFICE.

FRANK IRVING RUBRICIUS, OF NEW YORK, N. Y.

## SENSITIZING COMPOSITION FOR PHOTOGRAPHIC PAPER.

1,126,872.

Specification of Letters Patent.

Patented Feb. 2, 1915.

No Drawing.

Application filed May 31, 1913. Serial No. 770,962.

*To all whom it may concern:*

Be it known that I, FRANK I. RUBRICIUS, a citizen of the United States, and a resident of the borough of Manhattan, city, 5 county, and State of New York, have invented certain new and useful Improvements in Sensitizing Compositions for Photographic Paper, of which the following is a specification.

10 This invention relates to sensitizing preparations for use in photography, and has for its object the preparation of a sensitizing agent that may be used to sensitize thinner or more nearly transparent papers than it has heretofore been possible to sensitize with the preparations available, such paper, for instance, as Japanese tissue paper. Such papers are sufficiently transparent to permit the paper upon which they are 15 mounted to show through them, thereby making it possible to produce any tone desired by simply using a suitable color for the mount. Prints made upon such thin paper may also be glued upon glass plates 20 for use as lantern slides. In such instances the print upon the glass may be suitably colored. This is a great saving over the prevalent method of producing each lantern slide from a sensitized plate, for with my 25 sensitized tissue paper, only plain glass is necessary. A further advantage of such sensitized paper is the velvety appearance it presents. On account of this velvety appearance coarse retouching of the negative 30 does not show upon it.

A further advantage of my invention consists in the simplified manner in which paper sensitized with my preparation is developed, toned and fixed, thereby saving 35 time and money that would otherwise be expended for chemicals if the existing methods were pursued.

In carrying out the invention in its most preferred manner four solutions are prepared for the sensitizing agent, as follows: 40 The first solution is composed of ferric ammonium citrate, (green scales) 150 grains, preferably powdered gum arabic 15 grains and distilled water 1 ounce. The second 45 solution is composed of citric acid 60 grains

and distilled water 1 ounce. The third solution is formed of silver nitrate 70 grains and distilled water 1 ounce, and the fourth solution is composed of uranium nitrate 20 grains and distilled water 1 ounce. After 55 the ingredients of these solutions are dissolved the solutions are intermixed in the order above given, after which 30 drops of alcohol are added, care being taken that the preparation is continuously stirred as the 60 different solutions and alcohol are added.

The sensitizing preparation as thus formed may be used upon the paper or other material commonly used in photography and is not limited to any particular sizing 65 that may be applied upon the paper or other material. With my invention tissue papers may be sensitized which it has been impossible to sensitize with preparations heretofore used, thereby producing a new style of 70 paper which on account of its transparency and velvety surface is capable of many uses to which other papers cannot be put.

I prefer to use a sizing composed of Bermuda arrow-root 75 grains which is dissolved in 2 ounces of distilled cold water, after which 30 ounces of boiling water is added. To this solution is added glucose 20 grains and sodium phosphate dibasic 65 grains. This resultant solution is boiled for 80 about two minutes during which time it is stirred and then strained. The sizing thus formed is applied preferably by floating or immersing the paper or other material therein while warm, after which it is removed and quickly dried.

Paper containing my sensitizing preparation is developed and toned by the use of water only. It is fixed by the use only of a hypo bath, thereby producing a material 85 saving in time and money.

While I have described the carrying out of my invention in its most preferred manner I do not wish to limit the scope thereof to the particular ingredients and proportions herein set forth, for the various analogues of said ingredients may be substituted and different proportions may be used within certain limits without departing from the substance of this invention.

Having thus described my invention I claim—

A sensitizing preparation for use in photography containing a solution of ferric ammonium citrate (green scales), gum arabic, citric acid, silver nitrate, uranium nitrate, and alcohol substantially as described.

In testimony whereof I have hereunto set my hand in the presence of two witnesses.

FRANK IRVING RUBRICUS.

Witnesses:

S. THORNTON,  
O. B. KING.